# EUROPEAN PATENT APPLICATION

(11) **EP 1 449 648 A2**
(43) Date of publication of application: **25.08.2004**
(21) Application number: 04003556.0
(22) Date of filing: 17.02.2004
(51) Int. Cl.: B41C 1/00

(54) **Method of making a flexographic printing plate by lithographic transfer of an energy-curable composition**

(30) Priority: 18.02.2003 US 368262
(71) Applicant: Kodak Polychrome Graphics LLC, Norwalk, Connecticut 06851 (US)
(72) Inventor: Jianbing, Huang, Trumbull, CT 06611 (US)
(74) Representative: VOSSIUS & PARTNER

(57) **Abstract**

A method for making a relief printing plate, by using a lithographic printing plate to create ink-receptive areas on a receiver base. The relief printing plate has ink-receptive cured areas defining an image. The method comprises the steps of: a) imaging a lithographic printing plate precursor to produce a lithographic printing plate having ink-receptive image areas and ink-repellent non-image areas; b) applying a first curable composition to the lithographic printing plate, to form a coating of the first curable composition on ink-receptive image areas; c) contacting the coating to the receiver base to make an impression on the receiver base; and d) curing the impression on the receiver base to produce ink-receptive cured areas defining an image. In the practice of an embodiment of the invention, a modified rotary printing press may be employed to make a relief printing plate on a receiver base using a lithographic printing plate.

## Description

The present invention relates to methods for making relief printing plates, such as flexographic printing plates, from imageable lithographic printing plate precursors. The relief printing plates have ink-receptive cured areas defining an image (i.e., "image areas"), and ink-repellent non-image areas. In the practice of an embodiment of the invention, a modified rotary printing press may be employed to make a relief printing plate from a lithographic printing plate.

Relief printing plates are used in both flexographic and letterpress processes for printing on a variety of media, particularly for media which are soft and easily deformable, such as paper or plastic packaging materials, cardboard or other corrugated stock, film, foil, and laminates. Relief printing plates generally consist of raised image areas and depressed non-image areas. During printing, ink is transferred only from the raised image areas to the print media.

Historically, relief printing plates such as flexographic printing plates were formed from vulcanized rubber. Rubber was favored because it is resistant to harsh solvents, it has good ink transfer characteristics, high elasticity, and high compressibility. Rubber printing elements were originally made by vulcanizing the rubber material in a suitable mold. More recently, rubber printing elements have been made by direct laser engraving.

Relief printing plates are now generally made from photosensitive elements that are specifically designed for that purpose. The photosensitive elements that are used to make relief printing plates typically include a support layer, and one or more photosensitive layers comprising a photocurable composition including a polymer or prepolymer. Ideally the support layer is made from a dimensionally stable material, such as polyester film or an aluminum sheet

In making a relief printing plate from certain types of photosensitive elements, one side of the photosensitive layer is first exposed to an energy source (such as ultraviolet light) through the support to prepare a thin, uniform cured layer on the support side of the photosensitive layer. Then a masking device (such as a photographic negative) is placed over the photosensitive layer. The photosensitive element is then exposed to an energy source through the masking device, thereby causing exposed areas of the photocurable composition to harden, or cure. Unexposed and uncured portions of the photosensitive layer are then removed by a developing process, leaving the cured portions which define the relief printing surface.

Photosensitive elements comprising a top laser-ablatable mask layer have been reported. These types of plates may be made into relief printing plates without the use of a photographic negative or other separate masking device. Thus, "computer-to-plate" (CTP) processing may be achieved. In contrast to conventional methods that require a masking device, in a CTP method the preparation of a new masking device is not required when edits or modifications to the image are necessary. Modifications and edits to the image can be made on a computer, so that the CTP process advantageously saves time, labor and materials. Moreover, as compared with conventional masking devices such as photographic negatives, the photosensitive element has better dimensional stability, resulting in an improvement in reproducibility of the relief image and a corresponding improvement in printing quality.

Plates having an ablatable mask layer can be imaged by first imagewise exposing with laser radiation (generally under computer control) to selectively remove the mask layer in the exposed areas, and then overall exposing with an actinic radiation to cure the photosensitive layer in the unmasked areas. The remaining areas of the mask layer and the non-hardened portions of the photosensitive layer are then removed by one or more liquid development processes. Examples of such plates are described in U.S. Patent 5,705,310 to Van Zoeren, U.S. Patent 5,719,009 to Fan, U.S. Patent 6,020,108 to Goffing, *et al.,* and U.S. Patent 6,037,102 to Loerzer, *et al.* While plates having a laser-ablatable mask layer allow direct imagewise exposure with a laser and do not require a separate masking device, the mask layer removal process is cumbersome and generates chemical waste. It would be desirable to reduce or eliminate such a liquid development process in the processing of a relief printing plate.

U.S. Patent 4,410,562 to Nemoto, *et al*. reports a method for forming a cured resin coating having a desired pattern on the surface of a substrate. The method includes the steps of: applying a coating of a UV-curable resin to the surface of a substrate; procuring the coating; applying a printed layer in a predetermined pattern to the surface of the procured coating, using a light-insensitive, non-transparent printing ink; irradiating with UV light to cure the areas of the coating not covered by the printed layer; and removing the printed layer and the precured coating beneath the printed layer, to leave a cured resin coating, having a pattern complementary to the pattern of the printed layer, on the substrate. The reported method also requires removal of a portion of a photosensitive layer, and therefore wastes at least some of the UV-curable resin.

A stereolithographic technique for layer-by-layer buildup of a radiation-curable composition to yield a three-dimensional cured object is described in U.S. Patent 6,413,697 to Melisaris, *et al.* An alternative stereolithographic approach is reported in U.S. Patent 6,214,276 to Gelbart However, stereolithographic techniques are slow, often require a large bath of a curable liquid composition, and require repeated iterations in which a laser or other radiation source is rasterized or moved to form a pattern.

In one embodiment, the present invention provides a method for making a relief printing plate having ink-receptive cured areas on a receiver base, the method comprising the steps of: a) imaging a lithographic printing plate precursor to produce a lithographic printing plate having ink-receptive image areas and ink-repellent non-image areas, the ink-receptive image areas and ink-repellent non-image areas defining a first image; b) applying a first curable composition to the lithographic printing plate, to form a substantially uniform coating of the first curable composition on ink-receptive image areas; c) contacting the coating of the first curable composition to the receiver base to make an impression of the first curable composition on the receiver base; and d) curing the impression on the receiver base to produce a first cured layer, such that the first cured layer includes ink-receptive cured areas defining a second image corresponding to the first image.

The step of curing may be done by, for example, exposing the first curable composition to ultraviolet radiation or to a beam of electrons. The method may further include applying a coating of a second curable composition to ink-receptive image areas, contacting the coating of the second curable composition to the first cured layer to transfer the coating to the first cured layer, and curing the second curable composition on the first cured layer to produce ink-receptive cured areas including a second cured layer.

In a second embodiment, the invention provides a method for making a relief printing plate having ink-receptive cured areas on a receiver base, the method comprising the steps of: a) imaging a lithographic printing plate precursor to produce a lithographic printing plate having ink-receptive image areas and ink-repellent non-image areas, wherein the ink-receptive image areas and ink-repellent non-image areas define a first image; b) applying a first curable composition to the lithographic printing plate, to form a substantially uniform coating of the first curable composition on ink-receptive image areas; c) contacting the coating of the first curable composition to the receiver base to make an impression of the first curable composition on the receiver base; d) curing the impression on the receiver base to produce a cured layer, such that the cured layer includes ink-receptive cured areas defining an image corresponding to the first image; e) applying either the first curable composition or a second curable composition to the lithographic printing plate, to form a substantially uniform coating of the first or second curable composition on ink-receptive image areas; f) contacting the coating of the first or second curable composition to the cured layer, to transfer at least a portion of the coating of the first or second curable composition to the cured layer; g) curing the portion of the coating of the first or second curable composition on the cured layer, such that the cured layer includes ink-receptive cured areas defining an image corresponding to the first image; and h) repeating steps e) through g) to attain a desired relief depth for the ink-receptive cured areas of the cured layer; to produce the relief printing plate having ink-receptive cured areas defining an image corresponding to the first image.

This embodiment of the invention may be readily carried out in an automated fashion, such as by operating a rotary printing press adapted to carry out the steps of applying a coating of the first or second curable composition, contacting the coating to the receiver base, and curing the first or second curable composition on the receiver base. Practice of the method allows a relief printing plate to be built up in a layer-by-layer fashion, and does not require a developing step in which a significant quantity of a photosensitive layer of a photosensitive element is removed. Furthermore, the method requires less material, since little or no curable composition is wasted.

Fig. 1 shows a rotary printing press adapted for use in a method of the present invention.

### First Embodiment

In one embodiment, the present invention provides a method for making a relief printing plate having ink-receptive cured areas on a receiver base, the method comprising the steps of: a) imaging a lithographic printing plate precursor to produce a lithographic printing plate having ink-receptive image areas and ink-repellent non-image areas, the ink-receptive image areas and ink-repellent non-image areas defining a first image; b) applying a first curable composition to the lithographic printing plate, wherein the first curable composition wets ink-receptive image areas and does not wet ink-repellent non-image areas, to form a substantially uniform coating of the first curable composition on ink-receptive image areas; c) contacting the coating of the first curable composition to the receiver base to make an impression of the first curable composition on the receiver base; and d) curing the impression on the receiver base to produce a first cured layer, such that the first cured layer includes ink-receptive cured areas defining a second image corresponding to the first image.

### Imaging a Lithographic Printing Plate Precursor

In one step of the method, a lithographic printing plate precursor is imaged to produce a lithographic printing plate. As used herein, the term "lithographic printing plate" means an image-bearing planographic printing plate that has ink-receptive image areas and ink-repellent non-image areas. The phrase "image areas" is used herein to refer to individual halftone dots that make up an image on the printable surface of a lithographic printing plate. The phrase "non-image areas" is used herein to refer to areas on the printable surface of a lithographic printing plate that are not image areas.

A "lithographic printing plate precursor" is a non-image-bearing precursor that can be transformed into an image-bearing lithographic printing plate by suitable imaging and developing steps. A lithographic printing plate precursor generally includes a support and an imageable coating. In the practice of the present invention, suitable lithographic printing plate precursors include those that are intended for making wet printing plates (i.e., those that require a fount solution) and those that are intended for making waterless printing plates (i.e., those that do not require a fount solution). Both wet and waterless printing plates are widely known in the field.

The lithographic printing plate precursor includes an imageable coating. The imageable coating generally includes a radiation-sensitive composition that becomes either more soluble or less soluble in a developer upon exposure to radiation. In the practice of the invention, the imageable coating may be positive-working or negative-working. In the production of a lithographic printing plate, portions of the imageable coating are selectively exposed to radiation. After exposure, the imageable coating is generally developed to wash away the more soluble regions. The imageable coating that remains generally provides either ink-receptive areas or ink-repellent areas on the surface of the lithographic printing plate. Imageable coatings for lithographic printing plate precursors are widely known.

In printing plate precursors for wet printing plates, the support typically includes a hydrophilic surface, which is coated with the imageable coating. Generally, any material conventionally used as a support in a wet lithographic printing plate is suitable for the lithographic printing plate precursor used in the method. By way of example, a treated aluminum substrate is suitable as the support for the practice of the method. The surface of the aluminum substrate may be treated by metal finishing techniques known in the art including brush roughening, electrochemical roughening or electrograining, chemical roughening, anodizing, silicate sealing and the like. Aluminum substrates for lithographic printing plates are well-known in the field.

In printing plate precursors for waterless printing plates, the imageable coating typically includes a photosensitive layer and an ink-repellent layer (such as, for example, a silicone rubber layer or fluoropolymer layer) over the photosensitive layer and under any mask layer. After imagewise exposure the printing plate is developed. As a result of the developing process, the ink-repellent layer is removed from the non-hardened or solubilized areas of the photosensitive layer, and the ink-repellent layer remains in the hardened or non-solubilized areas of the photosensitive layer. During printing, ink adheres only to those areas of the printing plate not covered by the ink-repellent layer remaining after development Thus the plate can be printed without the need to use a fount solution. In contrast to printing plate precursors for wet printing plates, the support for a waterless printing plate may have an oleophilic surface. Generally, any material conventionally used as a support in a waterless lithographic printing plate is suitable for the lithographic printing plate precursor used in the method.

Ink-repellent layers in waterless printing plates are generally provided by amphiphobic (i.e., having both hydrophobic and oleophobic character) materials such as silicone polymers or fluoropolymers. Suitable waterless printing plate precursors including a support, a photosensitive layer and a top silicone-based layer are reported, for example, in U.S. Patent 5,061,598 to Abe, *et al.*, U.S. Patent 5,232,813 to Okuno, *et al.*, U.S. Patent 5,260,167 to Sasa, *et al.* U.S. Patent 5,786,125 to Tsuchiya, *et al.*, U.S. Patent 5,919,600 to Huang, *et al.*, U.S. Patent 5,955,238 to Yokoya, *et al.*, U.S. Patent 6,045,963 to Huang, *et al.*, and U.S. Patent 6,194,122 to Ichikawa, *et al.* Suitable waterless printing plate precursors including a support, a photosensitive layer and a top fluoropolymer-based layer are reported, for example, in U.S. Patent 6,130,026 to Bennett, *et al*.

A suitable support for the practice of the present invention may also be obtained by flood exposure of a commercially available radiation-sensitive flexographic printing plate precursor. The commercially available flexographic printing plate precursor could be flood-exposed on both front and back sides to initiate curing throughout An imageable coating as described herein could then be applied to provide a lithographic printing plate precursor useful in the practice of the invention. Another suitable support material is a rubber substrate as is known in the art, to which an imageable coating can be applied.

An optional adhesion promotion layer may be inserted between a silicone top layer and the photosensitive layer. One suitable adhesion promotion layer comprises an aminosilane, such as γ-aminopropyltriethoxy silane and γ-[N-(2-aminoethyl)amnopropyl] trimethoxysilane.

An optional protective layer may be laminated on top of a silicone layer to protect the silicone surface during storage and handling. A suitable protective layer is a thin polymeric film including polyesters such as polyethylene terephthalate, polyolefins such as polyethylene and polypropylene, and the like. The protective layer is designed to be easily removed without damaging the silicone layer surface either prior to or during processing.

By way of example only, the following waterless printing plate precursors are suitable as the lithographic printing plate precursor in the practice of the present invention: PEARLdry plates from Presstek, Inc. (Hudson, New Hampshire); SCORPION thermal waterless printing plates from Kodak Polychrome Graphics (Norwalk, Connecticut); TAN negative-working waterless plates and TAP positive-working waterless plates from Toray Industries (New York, New York).

By the step of imaging, the lithographic printing plate precursor is converted to a lithographic printing plate having ink-receptive image areas and ink-repellent non-image areas. By "ink-receptive," it is meant that the image areas will pick up a printing ink, either from a fount solution or from a waterless ink composition, during the printing process. In contrast, "ink-repellent" means that the non-image areas will not pick up the printing ink from a fount solution (in the case of a wet lithographic printing plate) or a waterless ink composition (in the case of a waterless lithographic printing plate).

One suitable method for imaging the lithographic printing plate precursor includes imagewise exposure to radiation. For imagewise exposure, a portion of the imageable coating is exposed to radiation to which the imageable coating is sensitive. The exposed portion becomes either more soluble or less soluble in a developer than an unexposed portion of the coating. The exposed portion corresponds to either image areas or non-image areas, the image areas and non-image areas together defining an image that is to be transcribed onto the lithographic printing plate precursor.

Imagewise exposure may be done by various methods common in the field, including analog and digital methods. Analog methods include techniques such as flood exposure to actinic radiation through an image-bearing separation transparency (e.g., a photographic negative). Alternatively, imagewise exposure may be accomplished by a digital method with computer control by rasterizing a laser across the imageable coating, and activating the laser beam at areas of the imageable coating that are to be exposed. In digital methods, the exposed and unexposed areas are determined by correspondence to a digital image that is generally stored on the controlling computer.

The step of imaging may further include the step of developing. The step of developing may include washing the lithographic printing plate, after imagewise exposure, in a suitable developer solution to remove either exposed portions or unexposed portions of the imageable coating. The step of developing generally exposes the hydrophilic surface underlying the imageable coating in non-image areas, for a wet printing plate; alternatively, the step of developing may expose an oleophilic surface underlying an imageable coating for a waterless printing plate. The choice of developer solution is generally determined by the nature of the imageable coating. Suitable developer solutions are well-known in the field of lithographic printing plates. Both organic-based and aqueous-based developers are available and suitable for the practice of the invention.

After the step of imaging, a lithographic printing plate is obtained. The lithographic printing plate has non-image areas in which an ink-repellent layer (which can be either hydrophilic or amphiphobic, depending on whether the plate is of the wet-type or waterless-type) is exposed, and image areas in which an ink-receptive coating persists. The ink-receptive image areas and ink-repellent non-image areas together define an image.

### Applying a Curable Composition to Ink-Receptive Image Areas

In another step of the method, a first curable composition is applied to the lithographic printing plate, to form a substantially uniform coating of the first curable composition on ink-receptive image areas.

### Curable compositions

Many curable compositions may be employed as the curable composition in the practice of the method. The phrase "curable composition" is used herein to mean a composition that can undergo a curing reaction initiated by heat or radiation, whereby the composition is transformed from an uncured state in which the composition is flowable and coatable, to a cured state in which the composition is at least partially hardened and flows less readily than in the uncured state. In general, a curable composition will include as one component at least one crosslinkable monomer or crosslinkable prepolymer, and the curing reaction will involve irreversible crosslinking of the crosslinkable monomer or prepolymer to make a cured material. As described below, the crosslinkable monomer or crosslinkable prepolymer may comprise, for example, an epoxide functional group or an ethylenically unsaturated functional group. A curable composition may also include other components such as a polymerization initiator, a binder, etc. Curable compositions in the practice of the invention may suitably be those that are curable or polymerizable by a free radical mechanism or those that are curable by a cationic mechanism, for example.

In general, the curable composition will be in a liquid form when applied. The curable composition may, however, be a solid at room temperature and become less viscous or liquid at elevated temperatures. Therefore, it may be necessary to heat the curable composition to achieve an appropriate viscosity before applying to the lithographic printing plate.

In order to avoid leaving the curable composition on ink-repellent non-image areas, it is desired that the curable composition have a relatively high viscosity when applied to the lithographic printing plate. The curable composition may suitably have a viscosity greater than about 100 cP in some embodiments, and may have a viscosity greater than about 500 cP in other embodiments.

Viscosity of the curable composition can be modified or increased by using reactive monomers or prepolymers having high molecular weights, or by adding polymeric binders of high molecular weight Polymeric binders can also be employed in the curable composition to achieve other desired properties of the curable composition or for the resulting cured material. Suitable polymeric binders include polyvinyl pyrrolidone or derivatives, such as those described in U.S. Patent 5,362,605 to Mitle, *et al.*; graft polymers, such as those described in U.S. Patent 5,204,222 to Gersdorf, *et al.*; block copolymer binders, such as those described in U.S. Patent 6,017,678 to Gries, *et al.*; diene copolymers, such as those described in U.S. Patent 5,281,510 to Sakurai, *et al.*; ionic polymer complexes, such as those described in U.S. Patent 6,159,658 to Tanaka, *et al.*; polyamides, such as those described in U.S. Patent 3,512,971 to Floss, *et al*; maleic copolymers; such as those described in U.S. Patent 5,859,134 to Reimers. A binder may suitably be included in the curable composition at a level up to 70 wt-% of the curable composition. The quantity of binder that should be included in the curable composition depends on a number of factors, including the molecular weight of the chosen binder and other parameters that dictate the effectiveness of controlling the viscosity of the curable composition.

Another method of increasing viscosity of the curable composition is to add a gelling agent. Gelling agents are typically capable of forming reversible links, such as for example hydrogen bonds or ionic bonds, with other components in the curable composition. Suitable gelling agents are reported, for example, in U.S. Patents 4,889,793 and 4,927,739 to Taniguchi, *et al.* Representative gelling agents include polyamides, polyesteramides, N-acyl. amino acid derivatives and the like. Complexing polymers reported in U.S. Patent 5,362,605 to Mirle, *et al.,* such as polyvinylpyrrolidone polymers and copolymers having molecular weight of 5 kDa to 100 kDa, may also suitably function as gelling agents.

A suitable curable composition will wet ink-receptive image areas and should not wet ink-repellent non-image areas of the lithographic printing plate. The term "wet" is used to indicate that the composition has relatively greater affinity for contact with the image areas than for contact with non-image areas, and will therefore preferentially coat the image areas.

Furthermore, the cured material obtained after a subsequent curing step described below should act as an ink-receptive material. In other words, upon curing of the curable composition, the ink-receptive image areas that are coated by the curable composition should become ink-receptive cured areas.

It is desirable that, after curing, the ink-receptive cured areas have good resistance to organic solvents such as alcoholic solvents typically used in flexographic printing inks and plate cleaners. Therefore, components of the curable composition should be chosen to provide this property in the cured material. Commonly used alcoholic solvents are ethanol, 2-propanol, n-butanol, and n-propanol. Resistance to such solvents can be achieved by adequate crosslinking in the cured materials, and selections of monomers and binders for the curable composition that are incompatible with alcoholic solvents.

The curable compositions of the present invention can be those curable or polymerizable by free-radical mechanisms. Such free-radical curable compositions typically contain a monomer or prepolymer component having a plurality of ethylenically unsaturated bonds available for crosslinking during a curing reaction. In the presence of free radicals, these unsaturated bonds quickly react with each other to form a three-dimensional network and thereby transform the curable composition into a cured material. By way of example, the unsaturated component may comprise methacrylate, acrylate or styrene. Ethylenically unsaturated components are well-known in the field of curable coatings for printing plates.

Free radicals can be generated to initiate curing by exposure of the curable composition to an energy source, oftentimes actinic radiation such as ultraviolet (UV) radiation, heat, or an electron beam. To enhance efficiency of free-radical generation, a free-radical initiator is generally included in the curable composition. The initiator is usually added in an amount ranging from 0.01 to 5% by weight of the total curable composition. Choice of free-radical initiators depends on the type of energy source to be applied during curing. Free-radical initiators are also well-known in the field of curable coatings for printing plates.

UV radiation is most commonly used energy source for curing. When such UV radiation is used, suitable initiators include the benzoin alkyl ethers, such as benzoin methyl ether, benzoin ethyl ether, benzoin isopropyl ether and benzoin isobutyl ether. Another class of initiators are the dialkoxyacetophenones exemplified by 2,2-dimethoxy-2-phenylacetophenone (available under the trade name IRGACURE 651 from Ciba-Geigy Corporation, Tarrytown, New York) and 2,2-diethoxy-2-phenylacetophenone. Still another class of initiators are the aldehyde and ketone carbonyl compounds having at least one aromatic nucleus attached directly to the carboxyl group. These initiators include, but are not limited to benzophenone, acetophenone, o-methoxybenzophenone, acetonaphthalene-quinone, methyl ethyl ketone, valerophenone, hexanophenone, alpha-phenyl-butyrophenone, p-morpholinopropiophenone, dibenzosuberone, 4-morpholinobenzophenone, 4'-morpholinodeoxybenzoin, p-diacetylbenzene, 4-aminobenzophenone, 4'-methoxyacetophenone, benzaldehyde, alpha-tetralone, 9-acetylphenanthrene, 2-acetylphenanthrene, 10-thioxanthenone, 3-acetylphenanthrene, 3-acetylindone, 9-fluorenone, 1-indanone, 1,3,5-triacetylbenzene, thioxanthen-9-one, xanthene-9-one, 7-H-benz[de]-anthracen-7-one, 1-naphthaldehyde, 4,4'-bis(dimethylamino)-benzophenone, fluorene-9-one, 1'-acetonaphthone, 2'-acetonaphthone, 2,3-butadione, acetonaphthene, benz[a]anthracene 7.12 diene, etc. Phosphines such as triphenylphosphine and tri-o-tolylphosphine are also operable herein as initiators.

Suitable curable compositions for the present invention also include compositions that are curable or polymerizable by cationic mechanisms. Compositions curable by cationic mechanisms typically comprise a cationic initiator, a source for generating active protons, and a component comprising a functional group that is crosslinkable by a cationic reaction. Electron beam-curable and UV-curable compositions are most common, but heat-curable compositions are also known.

The cationic initiators are compounds that liberate acidic species upon exposure to radiation. These acidic species then catalyze the crosslinking of the crosslinkable functional group. Typical initiators include onium salts such as sulfonium salts (e.g., triarylsulfonium salts), iodonium salts (e.g., diaryliodonium salts), and diazonium salts; and metallocenes. Alternatively, it is possible to thermally initiate cure through the use of onium or pyridinium salts that upon heating are known to afford cationic species capable of initiating a cationic cure.

The source for generating active protons may be, for example, an alcohol or polyol. The active protons facilitate the conversion of the initiator to a corresponding cationic species, which activates the cationic polymerization. The source for generating active protons may be, in some instances, a functional group (such as an -OH group) of the same component that provides the crosslinkable functional group.

The curable composition includes a component comprising a functional group that is crosslinkable by a cationic mechanism. The component is typically a polymerizable monomer or a polymerizable prepolymer. The crosslinkable functional group may be, for example, an epoxy or vinyl ether. The epoxide may be a cycloaliphatic epoxide, a glycidyl ester, glycidyl ether, or epoxidized alpha-olefin, for example. Other suitable components comprising a crosslinkable functional group include epoxidized diglycidyl ethers of bisphenol A, and novolac resins such as, for example, cresol epoxy novolac and phenol epoxy novolac. Suitable components may be obtained, for example, by epoxidation of polyhydric phenols such as bisphenol resins and novolac resins with epichlorohydrin, and compounds obtained by oxidation of linear olefin compounds and cyclic olefin compounds with peroxides.

The curable compositions suitable for the practice of the present invention may include compositions curable both by free radical and cationic means. Such "hybrid systems" are described, for example, in U.S. Patent 6,413,697 to Melisaris, *et al.*

The curable compositions may optionally contain additives that change or enhance properties of the curable compositions or of the resulting cured material. Additives are known in the art for use in radiation-curable compositions, and may include, for example, polymerization. inhibitors or stabilizers, antioxidants, antiozonants, and plasticizers.

To inhibit premature crosslinking during storage of the curable compositions of this invention, thermal polymerization inhibitors and stabilizers may be added. Such stabilizers are well known in the art, and include, but are not limited to, the following: hydroquinones such as hydroquinone monobenzyl ether, methyl hydroquinone, amyloxyhydroquinone, hydroquinone monopropyl ether; phenols, such as n-butylphenol, phenol, and phenolic-thio compounds; phenothiazine; phosphites; nitrobenzene; and mixtures thereof. Stabilizers may be included in an amount within the range from about 0.1% to about 3% by weight of the curable composition. These stabilizers are effective in preventing crosslinking of the curable composition during preparation, processing and storage.

The compositions may optionally contain up to about 30% by weight of an inert particulate filler. Such fillers include fine particulate material of inorganic material such as silica, magnesium carbonate, alumina, talc, clay, and titanium oxide. Such fillers can impart desirable properties to the curable compositions and reliefs on printing plates containing those compositions.

The compositions may optionally contain a plasticizer. Examples of suitable plasticizers include benzoates, phthalates, phosphates and sulfonamides.

### Methods of applying the curable composition

The step of applying the first curable composition may be performed by many application methods. The curable composition may be applied to the lithographic printing plate via the use of a suitable roller for carrying the curable composition, for example. Suitable rollers include rubber rollers with a flat surface and gravure rollers. Gravure rollers typically have recessed cells and are preferred for applying a uniform layer of the curable composition. Another suitable application method employs a Meyer bar or other wire-wound metering rod. The step of applying may also be performed using any conventional application methods, such as air doctor coating, blade coating, air knife coating, squeeze coating, reverse roll coating, transfer roll coating, gravure coating, kiss coating, cast coating, spray coating, dip coating, bar coating, extrusion coating, or die coating, for example.

Another suitable method of applying the curable composition onto the lithographic printing plate is by a screen printing method. In a screen printing method, a permeable sheet is placed in contact with the lithographic printing plate, and then the first curable composition is spread onto the permeable sheet by, for example, using a rubber roller. Once the curable composition has permeated the permeable sheet, the permeable sheet is then separated from the lithographic printing plate, leaving behind a substantially uniform coating of the curable composition on the ink-receptive image areas of the lithographic printing plate. (Optionally, the curable composition may be spread only onto the areas of the permeable sheet that cover ink-receptive image areas, to save material.) Suitable permeable sheets include those typically used in screen printing. Frames may optionally be used to support the permeable sheet with respect to the lithographic printing plate.

The curable composition may also be applied selectively to only ink-receptive image areas. A method of applying the curable composition selectively includes using an ink-jet printhead rasterized under computer control to dispense the curable composition only in ink-receptive image areas of the lithographic printing plate. Ink-jet printheads suitable for dispensing curable compositions include, for example, GALAXY and NOVA printheads available from Spectra, Inc. (Lebanon, New Hampshire).

The curable composition may be applied to any desirable thickness that may readily be cured during the curing step. A thickness of about 1 to about 10 microns, for example, is suitable.

The first curable composition is applied to form a substantially uniform coating of the first curable composition on ink-receptive image areas (i.e., individual halftone dots). By "substantially uniform," it is meant that the coating of the first curable composition should be of relatively even thickness and sufficiently free from defects (such as pinholes or voids) in the area to be coated so that the quality of an image will not be compromised. By way of example, the variation in the thickness of the layer would preferably be less than about 20% of the thickness of the layer, and more preferably the variation would be less than 10% of the thickness of the layer.

### Contacting the Receiver Base to Make an Impression of the Curable Composition

In another step, the coating is contacted to a receiver base to make an impression of the first curable composition on the receiver base. At least a portion of the coating that was applied to the lithographic printing plate is transferred to the receiver base to make the impression.

The receiver base includes a layer of a support material and may include additional layers. Materials that are suitable as the support layer include any material which is conventionally used to prepare flexographic printing plates. Flexible materials are commonly used as the support layer, and the support material is preferably a dimensionally stable material. Examples of suitable support materials include rubbers, polymeric films, fabrics such as fiberglass, and metals. Examples of particularly suitable dimensionally stable support materials are plates, sheets, and conical or cylindrical sleeves of metal such as steel, aluminum, copper, or nickel; plastics such as polyester or polyethylene terephthalate, polybutylene terephthalate, polyamide, and polycarbonate; woven and nonwoven fabrics such as glass fiber fabrics; and composite materials comprising glass fibers and plastics.

A suitable receiver base for the practice of the present invention may also be obtained by flood exposure of a commercially available radiation-sensitive flexographic printing plate precursor. The commercially available flexographic printing plate precursor could be flood-exposed on both front and back sides to initiate curing throughout.

The relief printing plates produced using the receiver base by the methods of the present invention may be suitable, for example, in flexographic printing. To work with existing flexographic printing presses, the receiver base may contain, in addition to the support layer, one or more ancillary layers that enhance functionality and performance of the resulting relief printing plate. For example, the receiver base may include layers to improve interlayer adhesion, to improve printing surface characteristics, and the like. Optional layers that may be added to the support to make an appropriate receiver base include, for example, an adhesion promotion layer or a primer layer.

For example, if the chosen support material for the receiver base does not have resilient properties typical of flexographic printing plates, such resilient properties may optionally be provided by an elastomeric primer layer coated on the support material. Useful primer layer compositions may include those described in U.S. Patent 5,061,598 to Abe, *et al.*, U.S. Patent 5,232,813 to Okuno, *et al.*, and U.S. Patent 5,260,167 to Sasa, *et al.* Alternatively, the primer layer may be a conventional thermoplastic coating or a thermoset coating. An example of a thermoplastic coating is polyvinyl alcohoL Examples of thermoset coatings include polyester-melamine coatings, acrylic melamine coatings, epoxy coatings, and polyisocyanate coatings.

A primer layer may provide not only a desired surface resilience, but also may offer a means for controlling thickness of the receiver base. By way of example only, a suitable overall thickness for. the receiver base is in the range of about 1 to about 3 mm.

In the step of contacting, the coating of the first curable composition is brought into contact with the receiver base, so that at least a portion of the coating that was applied to the lithographic printing plate is transferred to the receiver base to make an impression. Before contacting the coating to the receiver base, it may be useful to heat the lithographic printing plate to level the coating of the curable composition on the ink-receptive image areas of the lithographic printing plate.

Generally, the step of contacting should be carried out in such a manner as to leave a dean impression of the first curable composition on the receiver base. That is to say, the coating should be transferred to the receiver base without smearing, so that the act of transferring leaves an impression that corresponds to the first image.

The step of contacting may be done by bringing the lithographic printing plate into direct contact with the receiver base. Where the lithographic printing plate contacts the receiver base directly, the impression will be reversed left-to-right with respect to the first image on the lithographic printing plate. By way of example, one suitable method for contacting the lithographic printing plate to the receiver base is by mounting the lithographic printing plate and the receiver base onto respective cylinders of a rotary printing press, and then operating the press to bring the plate into contact with the base. The phrase "rotary printing press" is used herein to include printing presses having a plate cylinder, such as an offset printing press.

Alternatively, only the coating could come into direct contact with the receiver base. For example, the coating could be first transferred from the lithographic printing plate to a blanket cylinder, and then from the blanket cylinder to the receiver base. If this method of contacting is used, then the impression will be right-reading with respect to the image on the lithographic printing plate.

### Curing the Composition to Produce Ink-Receptive Cured Areas

After a portion of the coating is transferred to make the impression on the receiver base, the impression is cured to produce a first cured layer. As used herein, the term "curing" means at least partially hardening the curable composition so that it flows less readily than in the uncured state. The first cured layer includes ink-receptive cured areas defining a second image that corresponds to the first image. Where the lithographic printing plate contacted the receiver base directly to make the impression, the second image will be reversed left-to-right with respect to the first image.

In the step of curing, an energy source, to which the curable composition is sensitive, is applied. The step of curing may be done by, for example, exposing the curable composition to UV radiation or to a beam of electrons. Alternatively, heat may be applied to initiate curing, for an appropriate curable composition. Methods of curing are well-known in the field of curable compositions.

Before curing, it may be useful to heat the receiver base to level the impression of the first curable composition on the receiver base. Also, if the curable composition contains nonreactive volatile solvents, it may be desirable to remove such volatile solvents by moderate heating, prior to curing.

After curing, it may be useful to clean the receiver base to remove any loose material or debris that is not part of the first cured layer. Post-cure cleaning can be accomplished using a contact cleaning device such as a rotating brush such as is described in U.S. Pat No. 5,148,746 to Fuller, *et al.,* or by other suitable means.

The method may further include applying a second curable composition to ink-receptive image areas of the lithographic printing plate to form a substantially uniform coating, contacting the coating to the first cured layer to transfer a portion of the coating to the first cured layer, and curing the coating on the first cured layer to produce ink-receptive cured areas including a second cured layer. Any of the curable compositions described above may be useful as the second curable composition. The steps of applying, contacting, and curing may be carried out as described above.

By using a second curable composition that differs from the first cured composition, cured layers having different properties may be made. For example, the first cured layer may be suited to adhere to the receiver base, while the second cured layer may advantageously have better receptivity for a printing ink.

Alternatively, the second curable composition and the first curable composition may be identical. This embodiment may be useful, for example, in achieving layer-by-layer buildup of a relief image to produce a relief printing plate. The curable composition may be applied to the receiver base repeatedly and cured repeatedly, until a desired relief depth is attained.

The image areas of flexographic printing plates, in particular, require a certain range of surface hardness. Shore hardness is a commonly used measure for surface hardness for flexographic plates. Shore hardness may be measured with a durometer built according to standard test procedures as specified in ASTM D2240 00. For optimal durability as flexographic printing plates, the ink-receptive cured areas of the relief printing plates of the present invention have a type-A Shore hardness value in the range of 45 to 70.

### Second Embodiment

In a second embodiment, the invention provides a method for making a relief printing plate having ink-receptive cured areas on a receiver base, the method comprising the steps of: a) imaging a lithographic printing plate precursor to produce a lithographic printing plate having ink-receptive image areas and ink-repellent non-image areas, wherein the ink-receptive image areas and ink-repellent non-image areas define a first image; b) applying a first curable composition to the lithographic printing plate, wherein the first curable composition wets ink-receptive image areas and does not wet ink-repellent non-image areas, to form a substantially uniform coating of the first curable composition on ink-receptive image areas; c) contacting the coating of the first curable composition to the receiver base to make an impression of the first curable composition on the receiver base; d) curing the impression on the receiver base to produce a cured layer, such that the cured layer includes ink-receptive cured areas defining an image corresponding to the first image; e) applying either the first curable composition or a second curable composition to the lithographic printing plate, to form a substantially uniform coating of the first or second curable composition on ink-receptive image areas; f) contacting the coating of the first or second curable composition to the cured layer, to transfer at least a portion of the coating of the first or second curable composition to the cured layer; g) curing the portion of the coating of the first or second curable composition on the cured layer, such that the cured layer includes ink-receptive cured areas defining an image corresponding to the first image; and h) repeating steps e) through g) to attain a desired relief depth for the ink-receptive cured areas of the cured layer; to produce the relief printing plate having ink-receptive cured areas defining an image corresponding to the first image.

Steps a) through d) of the method may be performed as described above, using suitable materials as described above. Subsequently, either the first curable composition or a second curable composition is applied to the lithographic printing plate to form a substantially uniform coating of the first or second curable composition on ink-receptive image areas. The first or second curable composition is selected to wet ink-receptive cured areas and not wet ink-repellent non-image areas. The curable composition may be applied to any desirable thickness that may readily be cured during a subsequent curing step. A thickness of about 1 to about 10 microns, for example, is suitable. In the practice of the method, the steps of applying a first or second curable composition may be applied by any suitable method such as those described above, including a "screen printing" technique.

By using a second curable composition that differs from the first cured composition, cured layers having different properties may be made. For example, the first cured layer may be suited to adhere to the receiver base, while the second cured layer may advantageously have better receptivity for a printing ink. Alternatively, the second curable composition and the first curable composition may be identical.

After applying either the first or second curable composition to form a substantially uniform coating on ink-receptive image areas of the lithographic printing plate, the coating is contacted to the cured layer to transfer at least a portion of the coating to the cured layer. The portion that is transferred is then cured on the cured layer, to again produce a cured layer such that the cured layer includes ink-receptive cured areas. The ink-receptive cured areas define an image that corresponds to the first image (i.e., the image that was imparted to the lithographic printing plate in the imaging step).

In the step of curing, an energy source, to which the curable composition is sensitive, is applied. The step of curing may be done by, for example, exposing the curable composition to UV radiation or to a beam of electrons. Alternatively, heat may be applied to initiate curing, for an appropriate curable composition. Methods of curing are well-known in the field of curable compositions.

In the practice of the method, steps e) through g) are repeated to attain a desired relief depth for the ink-receptive cured areas of the cured layer. For each iteration, the thickness of the portion of the coating that is transferred may be any desirable thickness that can readily be cured during the curing step. A thickness of about 1 to about 10 microns, for example, is suitable.

This embodiment may be useful, for example, in achieving layer-by-layer buildup of a relief image to produce a relief printing plate. Each iteration increases the relief depth by approximately the thickness of the coating that is transferred. The method may be used to produce a relief printing plate having ink-receptive cured areas defining a second image corresponding to the first image. Steps e) and g) are repeated until a desired relief depth is attained for the ink-receptive cured areas of the second image.

Typical flexographic plates have a relief depth in the range 400 to 700 microns. The thickness built in each application of the curable compositions depends the rheology or viscosity of the curable compositions and application methods. Typically the layer thickness is in the range of 1 to 10 microns. Thus, to reach a relief depth of 400 micron, it may be necessary to build 40 to 400 layers by repeating steps e) through g) a suitable number of times.

For the practice of this embodiment, it may therefore be desirable to maintain a higher viscosity for the curable compositions, in order to increase the thickness added to the ink-receptive cured areas by each application of the curable compositions. Viscosity of the curable compositions may be changed or increased as described above. Another method of enhancing the rate of layer buildup is to include a particulate material in the curable compositions. Suitable particulate materials include those described above. Alternatively, the particulate material may be provided in the form of a microgel as described in U.S. Patent 4,956,252 to Fryd, *et al,* U.S. Patent 4,957,850 to Kusuda, *et al.,* or U.S. Patent 5,707,773 to Grossman, *et al*; particulate polymers described by U.S. Patent 5,736,298 to Koshimura, *et al.*; and latex particles as described in U.S. Patent 5,902,714 to Reimers, or U.S. Patent 6,210,854 to Grossman, *et al*. Particulate materials in the curable composition preferably have an average particle size in the range of about 0.5 to about 2 microns.

When the curable liquids are applied off-press, a suitable separating agent may be used to treat the lithographic printing plate before a subsequent application of a coating of a curable composition. Suitable separating agents include silicone fluids, for example. Use of such separating agents and related apparatus are described in U.S. Patent 5,676,053 to Schäfer.

After each curing step, it may be useful to dean the receiver base to remove any loose material or debris that is not part of the cured layer. Post-cure cleaning can be accomplished using a contact cleaning device such as a rotating brush such as is described in U.S. Pat No. 5,148,746 to Fuller, *et al.*, or by other suitable means.

Furthermore, the method may be readily carried out in an automated fashion, such as by operating a rotary printing press adapted to carry out the steps of applying a coating of a first or second curable composition to the lithographic printing plate, contacting the coating to the receiver base or cured layer to transfer a portion of the coating, and curing the transferred portion of the coating on the cured layer. The phrase "rotary printing press" is used herein to include printing presses having a plate cylinder, such as an offset printing press.

The curable compositions may be applied to the imaged lithographic printing plate by use of the rotary printing press, where the lithographic printing plate is mounted on the plate cylinder, and the curable composition is charged in the ink tray of the rotary printing press. A uniform ink layer on the ink-receptive image areas of the plate is obtained by running the press without feeding any paper.

One suitable method for contacting the lithographic printing plate to the receiver base is by mounting the lithographic printing plate and the receiver base onto respective cylinders of the rotary printing press, and then operating the press to bring the plate into contact with the base. Alternatively, only the coating could come into direct contact with the receiver base. For example, the coating could be first transferred from the lithographic printing plate to a blanket cylinder, and then from the blanket cylinder to the receiver base.

An energy source for curing may be mounted in appropriate relation to the cylinder on which the receiver base is mounted, so that the composition may subsequently be cured on the receiver base. The energy source may be activated either continuously or intermittently while the press is running. In the practice of this embodiment, it may be necessary to increase the gap between ink rollers and the plate cylinder and/or the gap between the plate cylinder and the blanket cylinder as the relief depth on the receiver base increases with the number of iterations.

Fig. 1 is a representation of a printing press adapted for the method. The printing press includes plate cylinder 100, impression cylinder 102, inking roller assembly 104, and energy source 106. Onto plate cylinder 100 is mounted an imaged lithographic printing plate 110 having ink-receptive image areas 112 and ink-repellent non-image areas 114. Onto impression cylinder 102 is mounted receiver base 120. As plate cylinder 100 rotates in the direction shown, a coating 116 of a curable composition is applied by inking roller assembly 104 to ink-receptive image areas 112. The coating 116 is brought into contact with receiver base 120 to make an impression 122. As the impression cylinder 102 rotates in the direction shown, impression 122 is exposed to radiation 108 from energy source 106, which initiates curing of the curable composition. A cured layer including ink-receptive cured areas 124 is formed, with ink-receptive cured areas 124 defining an image corresponding to the image on the lithographic printing plate. Several layers may be built up on the receiver base by continuing to operate the printing press. Layers may be added until a desired relief depth, which is the vertical distance from the major surface of an ink-receptive cured area 124 to the adjacent major surface of receiver base 120, is attained. In this manner, a relief printing plate can be made, comprising a relief image having ink-receptive image areas on a receiver base.

The accompanying figure is for illustrative purposes only, and is not limiting. Fig. 1 illustrates the method using a lithographic printing plate having an image area 112 that protrudes relative to non-image area 114. However, the methods of the invention may be carried out using imaged lithographic printing plates having image areas and non-image areas in the same plane, or using imaged lithographic printing plates having non-image areas that protrude relative to image areas (such as for some waterless plates).

In a variation of the method, a blanket cylinder (not shown) on the printing press may be employed. In this variation, an intermediate transferring of a portion of the coating to the blanket cylinder would take place, followed by transferring to the receiver base. Optionally, an intermediate receiver base could be mounted on the blanket cylinder. The intermediate receiver would accept a layer of the curable composition from the ink-receptive portions of the lithographic printing plate by an impression between the lithographic printing plate and the intermediate receiver. At least part of the impression of the curable composition would then be transferred to the receiver base on which the relief image is being built. For example, if an offset printing press is to be used, the lithographic printing plate is mounted on the plate cylinder, the intermediate receiver base is mounted on the blanket cylinder, and the relief image receiver base mounted on the impression cylinder.

Image areas of flexographic printing plates, in particular, require a certain range of surface hardness. Shore hardness is a commonly used measure for surface hardness for flexographic plates. Shore hardness may be measured with a durometer built according to standard test procedures as specified in ASTM D2240 00. For optimal durability as flexographic printing plates, the ink-receptive cured areas of the relief printing plates of the present invention have a type-A Shore hardness value in the range of 45 to 70.

It may also be desirable to coat the relief image with a suitable finish coat (also called a "capping layer" in the art of flexographic printing). The finish coat may provide properties such as increased surface hardness, better receptivity to a printing ink, enhanced ink transfer to the printing medium, or enhanced print quality.

This invention may take on various modifications and alterations without departing from the spirit and scope thereof. Accordingly, it is to be understood that this invention is not to be limited to the above-described, but it is to be controlled by the limitations set forth in the following claims and any equivalents thereof. It is also to be understood that this invention may be suitably practiced in the absence of any element not specifically disclosed herein.

In describing preferred embodiments of the invention, specific terminology is used for the sake of clarity. The invention, however, is not intended to be limited to the specific terms so selected, and it is to be understood that each term so selected includes all technical equivalents that operate similarly.

## Claims

1. A method for making a relief printing plate having ink-receptive cured areas on a receiver base, the method comprising the steps of:
(a) imaging a lithographic printing plate precursor to produce a lithographic printing plate having ink-receptive image areas and ink-repellent non-image areas, the ink-receptive image areas and ink-repellent non-image areas defining a first image;
(b) applying a first curable composition to the lithographic printing plate, wherein the first curable composition wets ink-receptive image areas and does not wet ink-repellent non-image areas, to form a substantially uniform coating of the first curable composition on ink-receptive image areas;
(c) contacting the coating of the first curable composition to the receiver base to make an impression of the first curable composition on the receiver base; and
(d) curing the impression on the receiver base to produce a first cured layer, such that the first cured layer includes ink-receptive cured areas defining a second image corresponding to the first image.

2. The method of claim 1 wherein the step of imaging a lithographic printing plate precursor includes imagewise exposing the printing plate precursor by a digital method.

3. The method of claim 1 wherein the step of imaging a lithographic printing plate precursor includes imagewise exposing the printing plate precursor by an analog method.

4. The method of any one of claims 1 to 3 wherein the step of imaging a lithographic printing plate precursor produces a waterless lithographic printing plate.

5. The method of any one of claims 1 to 4 wherein the first curable composition comprises an ethylenically unsaturated polymerizable component.

6. The method of any one of claims 1 to 5 wherein the first curable composition comprises a gelling agent to enhance the viscosity of the first curable composition.

7. The method of any one of claims 1 to 6 wherein the step of applying a first curable composition includes heating the lithographic printing plate.

8. The method of any one of claims 1 to 7 wherein the substantially uniform coating has a thickness in the range of about 1 to about 10 microns.

9. The method of any one of claims 1 to 8 wherein the receiver base comprises an elastomeric primer layer on a support layer.

10. The method of any one of claims 1 to 9 wherein the step of curing includes heating the receiver base.

11. The method of any one of claims 1 to 10 wherein the first curable composition includes an ultraviolet-sensitive component, and the step of curing includes exposing the coating of the first curable composition to ultraviolet light.

12. The method of any one of claims 1 to 10 wherein the first curable composition includes a component that is curable by electron irradiation, and the step of curing includes exposing the coating of the first curable composition to an electron beam.

13. The method of any one of claims 1 to 12, further comprising:
(e) applying a second curable composition to the lithographic printing plate, wherein the second curable composition wets ink-receptive image areas and does not wet ink-repellent non-image areas, to form a substantially uniform coating of the second curable composition on ink-receptive image areas;
(f) contacting the coating of the second curable composition to the first cured layer, to transfer at least a portion of the coating of the second curable composition to the first cured layer; and
(g) curing the portion of the coating of the second curable composition on the first cured layer to produce ink-receptive cured areas including a second cured layer.

14. The method of claim 13 wherein the second curable composition and the first curable composition are identical.

15. A method of any one of claims 1 to 12, further comprising:
(e) applying either the first curable composition or a second curable composition to the lithographic printing plate, wherein the second curable composition wets ink-receptive image areas and does not wet ink-repellent non-image areas, to form a substantially uniform coating of the first or second curable composition on ink-receptive image areas;
(f) contacting the coating of the first or second curable composition to the cured layer, to transfer at least a portion of the coating of the first or second curable composition to the cured layer;
(g) curing the portion of the coating of the first or second curable composition on the cured layer, such that the cured layer includes ink-receptive cured areas defining an image corresponding to the first image; and
(h) repeating steps (e) through (g) to attain a desired relief depth for the ink-receptive cured areas of the cured layer;
to produce the relief printing plate having ink-recepave cured areas defining an image corresponding to the first image.

16. The method of claim 15 wherein the receiver base comprises an elastomeric primer layer on a support layer.

17. The method of claim 15 or 16 wherein one of the first and second curable compositions comprises an ethylenically unsaturated polymerizable component.

18. The method of any one of claims 15 to 17 wherein one of the first and second curable compositions comprises a gelling agent to enhance the viscosity of the first or second curable composition.

19. The method of any one of claims 15 to 18 wherein one of the first and second curable compositions comprises a particulate material.

20. The method of any one of claims 15 to 19 wherein step (b) or step (e) includes heating the ink-receptive areas of the imaged lithographic printing plate.

21. The method of any one of claims 15 to 20 wherein step (d) or step (g) includes heating the receive base

22. The method of any one of claims 15 to 21 wherein the substantially uniform coating of the first or second curable composition has a thickness in the range of about 1 to about 10 microns.

23. The method of any one of claims 15 to 22 wherein one of the first and second curable compositions includes an ultraviolet-sensitive component, and step (d) or step (g) includes exposing the coating of the first or second curable composition to ultraviolet light.

24. The method of any one of claims 15 to 22 wherein one of the first and second curable compositions includes a component that is curable by electron irradiation, and step (d) or step (g) includes exposing the coating of the first or second curable composition to an electron beam.

25. The method of any one of claims 15 to 24 wherein the imaged litographic printing plate and the receiver base are each mounted on a separate cylinder of a rotary printing press, and wherein any of steps (b) though (h) includes operating the rotary printing press.

26. The method of claim 25 wherein an intermediate receiver base is mounted on another cylinder of the rotary printing press, and wherein step (c) includes:
transferring at least a portion of the coating to the intermediate receiver base; and
contacting the intermediate receiver base to the receiver base to make the impression.

27. The method of claim 25 wherein an intermediate receiver base is mounted on another cylinder of the rotary printing press, and wherein step (f) includes:
transferring at least a portion of the coating to the intermediate receiver base; and
contacting the intermediate receiver base to the cured layer, to transfer at least a portion of the coating to the cured layer.

28. The method of any one of claims 15 to 27 wherein the desired relief depth is in the range of about 400 to about 700 microns.

29. The method of any one of claims 15 to 28 wherein the ink-receptive cured areas of the relief printing plate are **characterized by** a Shore A hardness in the range of about 45 to about 70.

30. The method of any one of claims 15 to 29, further including the step of applying a separating agent to the ink-repellent areas so that the first or second curable composition does not wet ink-repellent non-image areas.

31. The method of claim 30 wherein the separating agent is a silicone fluid.

32. The method of any one of claims 15 to 31, further including the step of applying a finish coat to the relief printing plate.
